

## UNITED STATES PATENT OFFICE

2,395,846

## SENSITIZED PHOTOGRAPHIC EMULSION

Burt H. Carroll and John Spence, Rochester,  
N. Y., assignors to Eastman Kodak Company,  
Rochester, N. Y., a corporation of New Jersey

No Drawing. Application June 13, 1944,  
Serial No. 540,133

20 Claims. (CL. 95-7)

This invention relates to sensitized photographic emulsions and more particularly to spectrally (optically) sensitized emulsions.

It is known that the distribution of spectral sensitivity of certain spectrally sensitized emulsions can be altered and an increase of sensitivity obtained in some spectral region, by incorporating certain additional sensitizing dyes in the spectrally sensitized emulsions. (See United States Patents 2,158,882, dated May 16, 1939, and 2,159,565, dated May 23, 1939.) The effect thus obtained has come to be known as supersensitization. Supersensitization of certain spectrally sensitized emulsions can also be effected by incorporating certain substantially colorless heterocyclic bases, viz., those containing an amino group, in the spectrally sensitized emulsions. (See United States Patent 2,177,635, dated October 31, 1939.) Supersensitization differs from hypersensitization which involves treatment of finished films or plates, an operation which normally reduces the pAg and increases the pH of the emulsions, with consequent decreased stability.

We have now found a new method for supersensitizing spectrally sensitized emulsions, which not only does not reduce the stability of the emulsions, but is especially valuable as a means of giving panchromatic sensitized emulsions of high speed and exceptionally good color balance.

It is, accordingly, an object of our invention to provide new supersensitized photographic emulsions. A further object is to provide a process for preparing such emulsions. Still other objects will become apparent hereinafter.

In accordance with the invention, a photographic silver halide emulsion spectrally sensitized with one or more cyanine dyes is supersensitized by incorporating in the emulsion a heterocyclic nitrogen base selected from the group consisting of quinolones, benzothiazolones and thiazolinones. Exemplary of the quinolones are: 2(1)-quinolone (carbostyryl), the 4-alkyl-2(1)-quinolones, such as lepidone of the formula:



and the 1-alkyl-2(1)-quinolones, such as 1-methyl-2(1)-quinolone of the formula:



Exemplary of the benzothiazolones are the 2(1)-benzothiazolones, such as the compound of the following formula:



Exemplary of the thiazolinones are the 4-thiazolinones, such as 2-phenylamino-4-thiazolinone, e. g. the compound of the following formula:



or 2-ethylphenylamino-4-thiazolinone of the following formula:



We are aware that certain heterocyclic nitrogen bases containing a carbonyl group in the heterocyclic ring have been employed in photographic emulsions heretofore as color couplers. Typical of such heterocyclic nitrogen bases are homophthalimide which can be represented by the following formula:



and 3-hydroxy pyridine which can be represented by either of the following formulas:



50 The isoquinoline derivative (homophthalimide), however, is devoid of supersensitizing action. Three-hydroxy pyridine is likewise devoid of supersensitizing action. None of the pyridones show any marked supersensitizing action. Accordingly, isoquinolones and pyridones are specifically excluded from the purview of our invention.

The majority of cyanine dyes which are supersensitized by the heterocyclic nitrogen bases are characterized by the fact that the dyes produce 60 two types of sensitization depending upon con-

ditions. Such different types of sensitization are described by Leermakers, Carroll and Staud, J. Chem. Physics, 5, 878 (1937) and by G. Schwarz, Sci. et Ind. Phot. 10, 233 (1939). When a cyanine dye of this type is used as a sensitizer in low concentration, it exhibits a sensitizing maximum displaced out 20 to 55 mu, toward the red from the absorption maximum in ethyl alcohol solution. On increasing the concentration of the dye, or upon digesting the emulsion containing the dye in the lower concentration, or both, a second maximum of sensitization develops at longer wavelengths, which may be accompanied by an increase in total optical sensitization. In some cases, a decrease in sensitivity at the first maximum can be detected. These phenomena are consistent with the hypothesis of two states of the sensitizing dye in an equilibrium which is controlled by concentration. The heterocyclic nitrogen bases favor the formation of a second maximum which occasionally is appreciably displaced from the normal second maximum. The increase in sensitivity apparently corresponds to increased conversion of the dye to the state corresponding to the second maximum of sensitization. In some cases, the effect appears to correspond to a more complete conversion than has ever been obtained without a supersensitizer, and in any case the long wavelength sensitivity is better than can be obtained from the same concentration of dye without the heterocyclic nitrogen base.

The following are exemplary of the cyanine dyes which can be supersensitized in accordance with our invention:

3,3'-diethyl-9-methylthiacarbocyanine bromide  
9-ethyl-3,3'-dimethylthiacarbocyanine bromide  
5'-chloro-3,3',9-triethylthiacarbocyanine iodide  
5,5'-dichloro-3,3',9-triethylthiacarbocyanine bromide  
3,3'-diethyl-9-methyl-4,5,4',5' - dibenzothiacarbocyanine chloride  
3,3' - diethyl - 9 - methylselenathiacarbocyanine bromide  
5'-chloro-3,3'-diethyl-9 - methylselenathiacarbocyanine iodide  
3,3' - diethyl - 9 - methylselenacarbocyanine bromide  
5,5' - dichloro-3,3',9 - triethylselenacarbocyanine bromide

The sensitizing dyes can be employed in the same concentrations as would be used in the absence of the supersensitizer. Ordinarily from 10 to 30 mg. of dye per liter of emulsion will suffice to produce the optimum sensitizing effect. The methods of incorporating sensitizing dyes in emulsions are well known to those skilled in the art. Ordinarily it is preferable to dissolve the dye in a water-miscible solvent, such as methanol or ethanol before incorporating in the emulsion. One or more sensitizing dyes can be employed.

The amount of heterocyclic nitrogen base employed is not critical. Usually the full supersensitizing effect is developed at a concentration of from 0.10 to 0.50 gram per liter of emulsion. Practically none of the heterocyclic nitrogen bases has an appreciable effect on the pH of the emulsion. The heterocyclic nitrogen bases can be added to the emulsion with, before or after the sensitizing dye or dyes. More than one heterocyclic nitrogen base can be employed. The heterocyclic nitrogen bases are preferably, but not necessarily diluted with a water-miscible solvent,

such as methanol, before incorporation in the emulsion. The sensitizing dye or dyes and the heterocyclic nitrogen bases can be added to the emulsion at any convenient stage of its preparation, but preferably to the washed, finished emulsion.

The following examples will serve to illustrate results obtained in accordance with our invention.

#### Example 1

A fast negative gelatino-silver-bromide developing-out emulsion was sensitized with 3,3'-diethyl-9-methylthiacarbocyanine bromide (20 mg. per liter of emulsion) and to a portion of the spectrally sensitized emulsion was added 2(1)-quinolone (carbostyryl). A portion of the spectrally sensitized emulsion containing the quinolone and a portion of the spectrally sensitized emulsion without the quinolone were separately exposed, through red (Wratten 25) and minus blue (Wratten 12) filters, the latter giving a good measure of total optical sensitivity. The following results were obtained.

| 2(1)-quinolone (g. per liter of emulsion) | Red   |       | Minus blue |       | Fog  |
|-------------------------------------------|-------|-------|------------|-------|------|
|                                           | Speed | Gamma | Speed      | Gamma |      |
| None.....                                 | 115   | 1.41  | 435        | 1.52  | 0.11 |
| 0.5.....                                  | 255   | 1.27  | 795        | 1.30  | .10  |

#### Example 2

A fast negative gelatino-silver-bromide developing-out emulsion was sensitized with 3,3'-diethyl-9-methylselenacarbocyanine bromide (20 mg. per liter of emulsion) and to a portion of the spectrally sensitized emulsion was added 4-methyl-2(1)-quinolone (lepidone). A portion of the spectrally sensitized emulsion containing the quinolone and a portion of the spectrally sensitized emulsion without the quinolone were separately exposed, through red (Wratten 25) and minus blue (Wratten 12) filters. The following results were obtained.

| 4-methyl-2(1)-quinolone (g. per liter of emulsion) | Red   |       | Minus blue |       | Fog  |
|----------------------------------------------------|-------|-------|------------|-------|------|
|                                                    | Speed | Gamma | Speed      | Gamma |      |
| None.....                                          | 105   | 1.61  | 535        | 1.57  | 0.09 |
| 1.25.....                                          | 225   | 1.56  | 590        | 1.58  | .11  |

#### Example 3

A fast negative gelatino-silver-bromide developing-out emulsion was sensitized with 5,5'-dichloro-3,3',9-triethylselenacarbocyanine bromide (20 mg. per liter of emulsion), and to a portion of the spectrally sensitized emulsion was added 4-methyl-2(1)-quinolone. A portion of the spectrally sensitized emulsion containing the quinolone and a portion of the spectrally sensitized emulsion without the quinolone were separately exposed through red (Wratten 25) and minus blue (Wratten 12) filters. The following results were obtained:

| 4-methyl-2(1)-quinolone (g. per liter of emulsion) | Red   |       | Minus blue |       | Fog  |
|----------------------------------------------------|-------|-------|------------|-------|------|
|                                                    | Speed | Gamma | Speed      | Gamma |      |
| None.....                                          | 93.5  | 1.26  | 195        | 1.24  | 0.10 |
| 1.25.....                                          | 210   | 1.28  | 310        | 1.22  | .10  |

## Example 4

A fast negative gelatino-silver-bromiodide developing-out emulsion was sensitized with 3,3'-diethyl-9-methylthiacarbocyanine bromide (20 mg. per liter of emulsion), and to a portion of the spectrally sensitized emulsion was added 1-methyl-2(1)-quinolone. A portion of the spectrally sensitized emulsion containing the quinolone and a portion of the spectrally sensitized emulsion without the quinolone were separately exposed through red (Wratten 25) and minus blue (Wratten 12) filters. The following results were obtained:

| 1-methyl-2(1)-quinolone (g. per liter of emulsion) | Red   |       | Minus blue |       | Fog  |
|----------------------------------------------------|-------|-------|------------|-------|------|
|                                                    | Speed | Gamma | Speed      | Gamma |      |
| None.....                                          | 115   | 1.41  | 435        | 1.52  | 0.11 |
| 0.50.....                                          | 268   | 1.58  | 796        | 1.60  | .09  |

## Example 5

A fast negative gelatino-silver-bromiodide developing-out emulsion was sensitized with 3,3'-diethyl-9-methylthiacarbocyanine bromide (20 mg. per liter of emulsion), and to a portion of the spectrally sensitized emulsion was added 2(1)-benzothiazolone. A portion of the spectrally sensitized emulsion containing the benzothiazolone and a portion of the spectrally sensitized emulsion without the benzothiazolone were separately exposed through red (Wratten 25) and minus blue (Wratten 12) filters. The following results were obtained:

| 2(1)-benzothiazolone (g. per liter of emulsion) | Red   |       | Minus blue |       | Fog  |
|-------------------------------------------------|-------|-------|------------|-------|------|
|                                                 | Speed | Gamma | Speed      | Gamma |      |
| None.....                                       | 115   | 1.41  | 435        | 1.52  | 0.11 |
| 0.05.....                                       | 170   | 1.58  | 605        | 1.63  | .12  |

## Example 6

A fast negative gelatino-silver-bromiodide developing-out emulsion was sensitized with 3,3'-diethyl-9-methylthiacarbocyanine bromide (20 mg. per liter of emulsion), and to a portion of the spectrally sensitized emulsion was added 2-phenylamino-4-thiazolinone. A portion of the spectrally sensitized emulsion containing the thiazolinone and a portion of the spectrally sensitized emulsion without the thiazolinone were separately exposed through red (Wratten 25) and minus blue (Wratten 12) filters. The following results were obtained:

| 2-phenylamino-4-thiazolinone (g. per liter of emulsion) | Red   |       | Minus Blue |       | Fog  |
|---------------------------------------------------------|-------|-------|------------|-------|------|
|                                                         | Speed | Gamma | Speed      | Gamma |      |
| None.....                                               | 76    | 1.43  | 490        | 1.46  | 0.10 |
| 0.05.....                                               | 120   | 1.19  | 630        | 1.21  | .08  |

In a manner similar to that illustrated in the foregoing examples, other quinolones, benzothiazolones and thiazolinones can be employed to supersensitize emulsions spectrally sensitized with cyanine dyes. Some of the quinolones, e. g. 6-ethyl-1-methyl-2(1)-quinolone, while effecting supersensitization, cause some desensitization and must be employed with this fact in mind. In the above examples, the minus blue speed demonstrated whether or not there is a loss of total spectral (optical) sensitivity.

Our invention is primarily directed to the customarily employed gelatino-silver-halide developing-out emulsions, especially gelatino-silver-chlorobromide, gelatino-silver-bromide and gelatino-silver-bromiodide developing-out emulsions.

Emulsions prepared in accordance with our invention can be coated in the usual manner upon any desired support, such as cellulose nitrate support, cellulose acetate support, metal support, glass support or paper support.

The quinolones, benzothiazolones and thiazolinones referred to herein are named and numbered in accordance with current recommendations of Chemical Abstracts.

What we claim as our invention and desire to be secured by Letters Patent of the United States is:

1. A photographic silver halide emulsion spectrally sensitized with a cyanine dye, the emulsion containing, as a supersensitizer, a heterocyclic nitrogen base selected from the group consisting of 2(1)-quinolones, benzothiazolones and thiazolinones.

2. A photographic gelatino-silver-halide emulsion spectrally sensitized with a cyanine dye, the emulsion containing, as a supersensitizer, a heterocyclic nitrogen base selected from the group consisting of 2(1)-quinolones, benzothiazolones and thiazolinones.

3. A photographic gelatino-silver-halide developing-out emulsion spectrally sensitized with a cyanine dye, the emulsion containing, as a supersensitizer, a heterocyclic nitrogen base selected from a group consisting of 2(1)-quinolones, benzothiazolones and thiazolinones.

4. A photographic gelatino-silver-bromiodide developing-out emulsion spectrally sensitized with a cyanine dye, the emulsion containing, as a supersensitizer, a heterocyclic nitrogen base selected from the group consisting of 2(1)-quinolones, benzothiazolones and thiazolinones.

5. A photographic gelatino-silver-halide developing-out emulsion spectrally sensitized with a cyanine dye, the emulsion containing, as a supersensitizer, a 2(1)-quinolone.

6. A photographic gelatino-silver-halide developing-out emulsion spectrally sensitized with a cyanine dye which produces a maximum of spectral sensitivity in the emulsion at one concentration and at a higher concentration or upon digestion of the emulsion containing the dye at a lower concentration, produces a second maximum of spectral sensitivity at a wavelength longer than that of the first maximum, said emulsion containing, as a supersensitizer, a 2(1)-quinolone.

7. A photographic gelatino-silver-bromiodide developing-out emulsion spectrally sensitized with a cyanine dye which produces a maximum of spectral sensitivity in the emulsion at one concentration and at a higher concentration or upon digestion of the emulsion containing the dye at a lower concentration, produces a second maximum of spectral sensitivity at a wavelength longer than that of the first maximum, said emulsion containing, as a supersensitizer, a 2(1)-quinolone.

8. A photographic gelatino-silver bromiodide developing-out emulsion spectrally sensitized with a cyanine dye which produces a maximum of spectral sensitivity in the emulsion at one concentration and at a higher concentration or upon digestion of the emulsion containing the

dye at a lower concentration, produces a second maximum of spectral sensitivity at a wavelength longer than that of the first maximum, said emulsion containing, as a supersensitizer, a quinolone of the following formula:



9. A photographic gelatino-silver-halide developing-out emulsion spectrally sensitized with a cyanine dye, the emulsion containing, as a supersensitizer, a 2(1)-benzothiazolone.

10. A photographic gelatino-silver-bromiodide developing-out emulsion spectrally sensitized with a cyanine dye, the emulsion containing, as a supersensitizer, a 2(1)-benzothiazolone.

11. A photographic gelatino-silver-halide developing-out emulsion spectrally sensitized with a cyanine dye which produces a maximum of spectral sensitivity in the emulsion at one concentration and at a higher concentration, or upon digestion of the emulsion containing the dye at the lower concentration, produces a second maximum of spectral sensitivity at a wavelength longer than that of the first maximum, the emulsion containing, as a supersensitizer, a 2(1)-benzothiazolone.

12. A photographic gelatino-silver-bromiodide developing-out emulsion spectrally sensitized with a cyanine dye which produces a maximum of spectral sensitivity in the emulsion at one concentration and at a higher concentration, or upon digestion of the emulsion containing the dye at the lower concentration, produces a second maximum of spectral sensitivity at a wavelength longer than that of the first maximum, the emulsion containing, as a supersensitizer, a 2(1)-benzothiazolone.

13. A photographic gelatino-silver-bromiodide developing-out emulsion spectrally sensitized with a cyanine dye which produces a maximum of spectral sensitivity in the emulsion at one concentration and at a higher concentration, or upon digestion of the emulsion containing the dye at the lower concentration, produces a second maximum of spectral sensitivity at a wavelength longer than that of the first maximum, the emulsion containing, as a supersensitizer, a compound of the following formula:



14. A photographic gelatino-silver-halide de- 60

veloping-out emulsion spectrally sensitized with a cyanine dye, the emulsion containing, as a supersensitizer, a 4-thiazolinone.

15. A photographic gelatino-silver-bromiodide developing-out emulsion spectrally sensitized with a cyanine dye, the emulsion containing, as a supersensitizer, a 4-thiazolinone.

16. A photographic gelatino-silver-halide developing-out emulsion spectrally sensitized with a cyanine dye, the emulsion containing, as a supersensitizer, a 2-phenylamino-4-thiazolinone.

17. A photographic gelatino-silver-bromiodide developing-out emulsion spectrally sensitized with a cyanine dye, the emulsion containing, as a supersensitizer, a 2-phenylamino-4-thiazolinone.

18. A photographic gelatino-silver-halide developing-out emulsion spectrally sensitized with a cyanine dye which produces a maximum of spectral sensitivity in the emulsion at one concentration and at a higher concentration, or upon digestion of the emulsion containing the dye at the lower concentration, produces a second maximum of spectral sensitivity at a wavelength longer than that of the first maximum, the emulsion containing, as a supersensitizer, a 2-phenylamino-4-thiazolinone.

19. A photographic gelatino-silver-bromiodide developing-out emulsion spectrally sensitized with a cyanine dye which produces a maximum of spectral sensitivity in the emulsion at one concentration and at a higher concentration, or upon digestion of the emulsion containing the dye at the lower concentration, produces a second maximum of spectral sensitivity at a wavelength longer than that of the first maximum, the emulsion containing, as a supersensitizer, a 2-phenylamino-4-thiazolinone.

20. A photographic gelatino-silver-bromiodide developing-out emulsion spectrally sensitized with a cyanine dye which produces a maximum of spectral sensitivity in the emulsion at one concentration and at a higher concentration, or upon digestion of the emulsion containing the dye at the lower concentration, produces a second maximum of spectral sensitivity at a wavelength longer than that of the first maximum, the emulsion containing, as a supersensitizer, the compound having the following formula:



BURT H. CARROLL.  
JOHN SPENCE.

**Certificate of Correction**

Patent No. 2,395,846.

March 5, 1946.

BURT H. CARROLL ET AL.

It is hereby certified that error appears in the printed specification of the above numbered patent requiring correction as follows: Page 2, second column, line 41, Example 2, for "quinoline" read *quinolone*; and that the said Letters Patent should be read with this correction therein that the same may conform to the record of the case in the Patent Office.

Signed and sealed this 21st day of May, A. D. 1946.

[SEAL]

**LESLIE FRAZER,**  
*First Assistant Commissioner of Patents.*